

Oct. 26, 1937.

G. EMBERG

2,096,888

PROCESS OF SATURATING FIBROUS CONDUITS

Original Filed May 27, 1932



INVENTOR  
GEORGE EMBERG

BY *Finn Liley*  
ATTORNEY

## UNITED STATES PATENT OFFICE

2,096,888

## PROCESS OF SATURATING FIBROUS CONDUITS

George Emberg, Chicago, Ill., assignor to The Barrett Company, New York, N. Y., a corporation of New Jersey

Original application May 27, 1932, Serial No. 613,937. Divided and this application August 13, 1935, Serial No. 35,991

8 Claims. (Cl. 91—70)

This invention is directed to the saturation of absorbent conduits, and more particularly, to a batch process of saturating and impregnating fibrous conduits employed to conduct and protect 5 underground cables, telephone lines, electric light and other conductors and for the formation of drain pipes utilized for the discharge of corrosive liquids to render them substantially waterproof and resistant to abrasion, corrosion, and conditions encountered underground by fibrous conduits.

The fibrous bases of the conduits for the preferred embodiment of my invention may be prepared in any well known manner. For example, 15 newsprint and paper pulp or other fibrous material may be beaten in the usual paper beaters and the resultant stock screened and then pumped to paper cylinder machines and there formed into wet felts or paper. The wet paper may be wound 20 about a cylindrical tube or mandrel to produce a wet conduit of proper thickness. This conduit may be dried in kilns to remove the major portion of its moisture content. The fibrous base may, of course, be prepared in other known manner. 25 Such conduits are made in several sizes, varying from 2 inches to 6 inches or larger in external diameter, have an average wall thickness of approximately  $\frac{1}{8}$  of an inch and are usually produced in 5, 6, and 8 foot lengths. The wall thickness of the conduits may, of course, be greater or less than  $\frac{1}{8}$  of an inch and other dimensions 30 may vary. As they come from the drying kilns, they usually contain from 5 to 8 per cent moisture, although considerably more than 8 per cent moisture may, on occasion, be found present.

The porosity or absorptive characteristics of the walls of fibrous conduits may vary within wide limits from a very dense wall of density corresponding to hard wood and exceedingly difficult to saturate with low carbon water gas tar pitch or even with other waterproofing material, such as asphalt, to a porous open wall similar in density to that of roofing felt, which will readily absorb bituminous saturants. Samples of present 40 commercial fibrous conduits have been tested and found to vary from substantially less than 1 cc. of voids per gram of tube wall to 2.8 or more cc. of voids per gram of tube wall. To determine the cubic centimeters of voids per gram of tube wall, a small sample of tube wall (say 2" x 5") is dried for one hour at 100° C., cooled, desiccated, and thereafter weighed. It is then immersed in kerosene, maintained at a temperature of 25° C., for 18 hours. Thereafter, the sample is removed 50 from the kerosene, drained in vertical position for

30 seconds, and again weighed. The difference in weight represents the kerosene absorbed. This difference in weight in grams, divided by the specific gravity of the kerosene, corresponds to the cubic centimeters of kerosene absorbed. This 5 volume in cubic centimeters, divided by the original weight in grams, gives the voids in cubic centimeters per gram.

The fibrous conduits, as they come from the drying kiln, containing from 5 to 8 per cent of moisture, have heretofore commonly been impregnated with water gas tar pitch by immersing them in tanks of molten pitch maintained at atmospheric pressure or pressure above atmospheric and at a temperature of 300° F. or upwards. The conduits have in many cases been allowed to soak in the molten pitch for from 7 to 12 hours, then withdrawn, and permitted to drain to remove excess saturant therefrom.

This process of saturating fibrous conduits, it 20 will be noted, requires the soaking of the conduits for long periods of time to obtain satisfactory penetration of the saturant throughout the walls of the conduit. In the practice of the process, numerous difficulties are encountered, 25 among the most important of which may be mentioned—

(1) Foaming of the pitch during the saturation of the conduits with consequent loss of volatile oils from the pitch and restriction of the 30 amount of pitch absorbed by the fibrous walls. This, I have found, may largely be attributed to the moisture content of the fibrous tubes;

(2) Building up of the "free carbon" content of the pitch due to the prolonged maintenance of large bodies of pitch in which the conduits are immersed under heat, resulting in decomposition of the pitch. Increase in the "free carbon" content of the pitch decreases the penetrability of the saturant and also results in carbon deposits on the walls of the conduit, preventing entrance of the saturant thereto and resulting in defectively saturated conduits, i. e., conduits having "white spots" within the walls. The term "free carbon" is used in the sense common in the coal tar industry to indicate material contained in the bituminous saturant which is insoluble in benzol or carbon bisulfide. It is commonly determined as described by Weiss (Journal of Industrial and Engineering Chemistry, vol. 10, 1918, pages 736 and 820, Test D5). It comprises high-molecular carbon compounds of low solubility, carbon, and other insoluble material;

(3). Unsatisfactory saturation of the conduits due to the fibrous walls not absorbing sufficient 55

saturant to render them substantially waterproof. Conduits which are not adequately saturated do not attain maximum strength and resistance to deflection or deformation; and

- 5 (4) In the case of saturation of conduits under substantially atmospheric pressure, or under higher pressures, a substantial fire hazard may exist. This is especially the case where increased pressure is produced by air pressure on the saturant and where incompletely covered and protected saturating tanks are used.

Due to long time immersion of the organic or fibrous bases in hot saturant, charring or burning of the organic bases frequently takes place.

- 15 Water gas tar pitch has heretofore largely been employed as the saturant for fibrous conduits. As is well known, water gas tar pitch is obtained by distilling tar derived from carburetted water gas made by enriching blue gas with products 20 of pyrogenic decomposition of petroleum oils. The oils constitute the chief source of tar present in the carburetted water gas. Water gas tar pitch is, therefore, essentially of petroleum origin and it is recognized that water gas tar pitch differs materially in composition from other pitches, particularly coal tar pitches derived from the distillation of tar obtained from coal distillation gases. Water gas tar pitch has been employed 25 for saturating fibrous conduits largely because of its relatively low "free carbon" content (about 30 2 to 7 per cent); its improved waterproofing properties as compared with asphalt; and its capability to protect the fibrous base against molds and fungi. While in some cases asphalts 35 have been employed for the saturation of conduits, generally speaking, they are less satisfactory than pitch in that they are less waterproof and do not effectively withstand and protect 40 against molds and fungi and other cellulose destroying organisms.

In order to satisfactorily protect cables and other electrical conductors, it is important that the conduit be substantially waterproof, resistant to abrasion and soil pressures, and capable of 45 withstanding underground conditions and not punctured or broken by the soil and debris surrounding it. One of the tests to which conduits are subjected to determine their waterproofness is to immerse them in distilled water, maintained at 50 a temperature of approximately 77° F. for 48 hours, then ascertain the percentage increase in the weight of the conduit and thus arrive at the amount of water absorbed thereby. Present 55 conduits, saturated with water gas tar pitch, have been tested in this manner and many have been found to absorb in the neighborhood of 12 per cent of water. At the present time, it is generally recognized that a conduit which, upon immersion 60 for 48 hours in distilled water maintained at a temperature of approximately 77° F., will absorb not more than 6 per cent moisture represents a satisfactory waterproof conduit; a conduit absorbing not more than 4 per cent moisture under 65 these conditions is regarded as eminently satisfactory. It should be noted that as indicated hereinabove, many of the saturated fibrous conduits now made, when subjected to the waterproofness test briefly described above, show an 70 absorption of moisture substantially in excess of 4 per cent, many of them absorbing 12 per cent and more moisture. In general, the lower the water absorption, the more satisfactory is the product.

75 In the impregnation of porous articles with

bituminous saturant, two of the factors which tend to prevent satisfactory saturation are—

1. Air in the pores or voids, and
2. Moisture on the fibers or other solid surfaces and as vapor in the pores.

Air and water vapor in the pores of the material tend to prevent entrance of the saturant, and water on the material surfaces tends to prevent wetting of the surfaces by the saturant.

When saturation is attempted at atmospheric pressure, the major portion of the water may be removed by long soaking in the hot saturant at a temperature above the boiling point of water. The escaping steam carries with it some air. The removal of water by this means is time-consuming and air is not completely removed. By the heretofore commonly practiced methods of saturation, therefore, the voids of the saturated article are incompletely filled with saturant.

If it is attempted to improve the degree of 20 saturation by applying pressure, some improvement is found, but saturation is still imperfect. The effect of pressure is, by forcing additional saturant into the material, to compress residual air and water vapor in the pores, even to the extent of somewhat compressing, densifying, and deforming the walls of the saturated article. On release of pressure, the compressed air and water vapor expand, forcing pitch out from the material, thereby reducing the degree of saturation 30 and even distribution of the saturant.

My invention largely or entirely eliminates these disadvantages and produces an article the voids of which are nearly or completely filled with saturant. Such articles are more resistant to 35 water-absorption, abrasion, deflection, and deformation. In the process of my invention, the walls of the fibrous conduits are not subjected to pressure or other conditions which would cause densification or compression of the tube walls 40 with consequent increased resistance to absorption of saturant, but on the contrary the pores or voids are evacuated during saturation, materially increasing the absorbing capacity of the tube wall. Moreover, my process as compared 45 with prior procedures minimizes the pumping and other handling of saturant.

In accordance with this invention a batch of conduits is first dried. The drying of the conduits may be accomplished in any desired manner, as for example, by permitting the conduits to soak in hot saturant or by subjecting them to heat out of contact with the saturant or by soaking the conduits in the saturant which will be employed for saturating the conduits. The drying of the conduits may be carried out under vacuum which may be gradually increased to a maximum, say 28 to 29 inches of mercury, and the conduits held at this vacuum while heated for a period long enough to remove substantially all 50 water, water vapor, and air from the voids.

A batch of the dried conduits is then immersed in a body of saturant. After immersion vacuum is pulled on the body of saturant. A vacuum of from 17 to 29 inches of mercury may be maintained on the saturant. The higher the vacuum attained the more effective is the removal of air and water from the voids and the more complete is the absorption of saturant.

In the case where the conduits are soaked in 70 the body of saturant employed for the saturation, when the soaking has proceeded to the point where the conduits are substantially completely dried, a vacuum is then pulled on the body of saturant containing the conduits.

The immersion of the conduits in the saturant prior to pulling the vacuum thereon results in the entire area of the conduit walls contacting with the saturant when the body of saturant is subjected to vacuum. Hence impregnation of the conduits by capillarity takes place slowly over the entire area of the walls of the conduits, giving substantially complete impregnation. The maintenance of vacuum conditions during impregnation permits removal of residual air and moisture in the conduit voids, and facilitates entry of saturant into the evacuated voids, with consequent increased absorption of saturant by the conduits. The time of soaking of the conduits in the saturant while maintained under vacuum may vary from about forty-five minutes to two hours, depending on the density of the fibrous base of the conduits, the saturant employed, etc.

While the conduits are permitted to soak in the saturant the vacuum is broken. Interruption of the vacuum may be gradual by admitting air or other inert gas to the saturating tank so that the pressure above the saturant gradually builds up to atmospheric while the conduits are immersed in the saturant. Increase in pressure of the saturant containing immersed conduits results in the forcing of the maximum amount of saturant into the voids of the conduits.

The conduits may be permitted to soak in the saturant at atmospheric pressures or pressures above atmospheric and then removed.

In the practice of this process a body of saturant may be maintained in a suitable container equipped with vacuum producing means and successive batches of conduits introduced and immersed in the body of saturant, vacuum pulled on the body of saturant after immersion, and after saturation is completed the vacuum interrupted and the saturated conduits withdrawn and a fresh batch of conduits introduced thereunto and the steps repeated. Removal of the saturant from the container is not required. Additional saturant may be added to the body in the container from time to time to replace the saturant absorbed by the conduits. It will be noted, therefore, that the process of this invention minimizes the handling of the saturant.

Coal tar pitch, preferably a pitch having a melting point of from 140° to 180° F. may be used as a saturant in the process of this invention. Pitch of a melting point as high as 225° F. may be employed in special cases, e. g., with conduits having large size voids. Preferred pitches having melting points of from 140° to 180° F. or higher will have a "free carbon" content of from 5 to 9 per cent, and may be employed to saturate fibrous conduits in accordance with this invention resulting in a more waterproof, stronger and otherwise improved conduit. Best results are obtained using pitches having a relatively low free carbon content. Pitches of "free carbon" content up to from 15 to 25 per cent, or even higher may be used to give commercially satisfactory saturation; preferably such high "free carbon" pitches are employed to saturate products having unusually open structure.

Preferably coal tar pitch made by a vacuum distillation process, such for example as disclosed in Patent No. 1,759,816, granted May 20, 1930, or other processes minimizing decomposition of the tar undergoing distillation, is employed as the saturant. Pitches made by a low temperature vacuum distillation process are characterized by low "free carbon" content and I have found that such pitches are particularly suitable as the sat-

urant for fibrous conduits. For example, such a pitch of 149° F. melting point (water bath) had a "free carbon" content of from 5 to 9 per cent; such pitch of 158° F. melting point (water bath) had a "free carbon" content of from 5 to 9 per cent; such pitch of 226° F. melting point (air bath) had a "free carbon" content of from 11 to 15 per cent; and such pitch of 291° F. melting point (air bath) had a "free carbon" content of from 16 to 21 per cent. Pitches produced by distilling tar not under vacuum but by continuously heating the tar and then passing the heated tar into a vapor box where the vapors separate from the pitch have considerably higher "free carbon" contents for the same melting point pitch, e. g., pitch produced in this manner having a melting point of 149° F. (water bath) had a "free carbon" content of from 11 to 13 per cent; a pitch of 158° F. melting point (water bath), had a "free carbon" content of from 10 to 14 per cent; a pitch of 226° F. (air bath) had a "free carbon" content of from 19 to 23 per cent; and a pitch of 291° F. melting point had a "free carbon" content of from 33 to 37 per cent. The "free carbon" content will depend largely on the melting point of the pitch and the "free carbon" content of the tar used to make the pitch. Coke oven tar generally will not run much above 5 per cent "free carbon"; 1 per cent "free carbon" content is very low for such tars.

The use of a pitch made by a vacuum distillation process for saturation has a two-fold advantage:

(1) In its manufacture, this pitch is distilled under vacuum and consequently at a lower temperature than would be needed to produce a pitch of the same melting point by the usual methods of distillation. This low temperature causes minimum decomposition and hence minimum "free carbon" formation in the pitch. Low "free carbon" content is an aid in effecting complete penetration and saturation of porous material.

(2) In its manufacture, the pitch has been subjected to temperature and vacuum conditions such as to insure the substantially complete removal of oils which would be volatile under the conditions maintained in the saturating operation of my invention. Such pitches will be substantially non-volatile at the temperature and vacuum conditions encountered in the saturating operation, and consequently, will suffer minimum or substantially no loss from volatilization during saturation. Owing to low volatilization losses, increase in "free carbon", as well as change in melting point, during saturation will be reduced to a minimum.

Other methods of manufacture, such as steam- or inert-gas-distillation, which effect distillation at relatively low temperatures, will yield desirable pitches for my process for the reasons outlined above.

In the drawing, the single figure is a vertical section partly in elevation of one form of apparatus for practicing the process of this invention.

Referring to the drawing, reference numeral 1 indicates a saturating tank or container, preferably of an over-all height of approximately 5 feet in excess of the length of the conduits or tubes to be treated. A cover 2 pivoted at 2' has a flange 3 arranged to be bolted or otherwise secured against vacuum leakage, as indicated at 4, to flange 5 on container 1. In lieu of bolting the cover to the container, flanges 3 and 5 may be ground to form a gas-tight joint when

properly assembled. Cover 2 has a hook or eye 6 to permit ready removal from and placement onto the tank 1.

The bottom of the container is shown provided 5 with a steam jacket 7 having steam inlet 8 and outlet 9 for supplying heat to the tank 1, although other heating means may be employed. At a point near the base of the container, a screen or other suitable support 11 is provided for a basket 10 12 containing the conduits 13 to be impregnated. Heat insulating material (not shown) may be disposed about the tank and other parts of the apparatus to reduce heat losses therefrom.

Saturant is supplied to the tank 1 through 15 valve-controlled pipe 14, disposed at the base of the tank. An over-flow pipe 15 is connected to a side wall of the tank near the top thereof. This pipe may communicate with a storage tank (not shown) for the saturant. If desired saturant may flow under gravity into tank 1 through 20 a valve controlled inlet pipe 10. Extending through the side of tank 1, through a gas-tight packed joint, is a pipe 16. This pipe is communicably connected with condenser 17 having inlet 25 18 and exit 19 for cooling water or other medium. A suction pump 21 of any suitable type is connected by pipe 22 with the trap 26 into which leads section 23 of pipe 16. A baffle 28 in the trap 26 prevents flow of liquid through the trap 30 into the vacuum line 22. Pipe 24 connects trap 26 with oil and water collector 25. Valves 27 are disposed in pipe lines 16, 22, and 24 to control flow therethrough.

A conveyor chain or rope 31, provided with a 35 hook or engaging means 32, is designed to run over a guide pulley 33. This conveyor chain can be operated manually or by power driven means to lower a basket of conduits or tubes into the saturant and the chain is then removed from the saturant in tank 1, cover 2 secured in position and the saturation carried out as hereinabove described. Upon the completion of the saturating operation, cover 2 may be opened and the hook on the chain placed in engagement with the eye 45 34 on the perforated basket 12 containing the fibrous conduits, and this basket withdrawn from the saturating tank.

In operation, the fibrous conduits to be saturated are placed in the perforated basket 12, 50 preferably, but not necessarily, in vertical position, and the basket then immersed in the saturant. As indicated in the drawing, the tank 1 has an over-all height such that a considerable open space is provided above the top of the conduits. The conduits may be permitted to soak in the saturant to effect the drying thereof, steam being passed through the jacket 7 to facilitate drying. In lieu of drying the conduits at atmospheric pressure, cover 2 may be seated on the saturating tank and the vacuum pump-started. Simultaneously with the vacuum to which the conduits are subjected, the container or saturating tank may be heated by passing steam through the jacket 7. Instead of drying the conduits by soaking them in the saturant in tank 1, the conduits may be dried in any other suitable manner.

After the drying is completed, the dried conduits, if not already immersed in the saturant, 70 are then immersed. Vacuum is then pulled on the saturant and the conduits permitted to soak in the saturant while maintained under vacuum. Upon completion of the saturating operation, the vacuum is interrupted, cover 2 opened and the conduits withdrawn. A fresh batch of dry con-

duits may then be inserted in the saturating tank 1 and the steps repeated.

In the drawing I have shown tubes or conduits treated in a vertical position. By suitable changes in the apparatus I may treat them equally effectively in a horizontal position.

I have found as a result of work performed, a conduit having about 1.6 cc. of voids per gram of tube wall saturated in accordance with my invention with coal tar pitch (e. g. containing 10 6-12% free carbon) will absorb an amount of saturant equal to more than 200 per cent of the weight of the dry unsaturated base. In saturating very dense fibrous conduits, for example, conduits having approximately 0.67 cc. of voids per 15 gram of tube wall, with coal tar pitch or other bituminous saturant, the amount of saturant absorbed will be found to be as much as eighty per cent by weight of the dry unsaturated base.

Prior processes of saturating fibrous conduits even with low or lower free carbon content water gas tar pitch have not given anywhere near such high percentage impregnation. Using asphalt as the impregnating medium or saturant in accordance with this invention, much greater amounts 25 of saturant may be introduced into the conduit walls as compared with the saturation of conduits with asphalt in accordance with prior procedures. Asphalt, as is well known, may contain less than 1% free carbon or may contain no 30 free carbon. It will be noted that the process of this invention results in conduits having voids or pores substantially completely filled with coal tar pitch or other saturant employed, and has the coal tar pitch or other saturant covering the 35 fibres and bonding with the pitch in the voids. Hence the fibrous base is effectively waterproofed to protect it against corrosion, abrasion and soil pressures. Conduits resulting from the practice of the process of this invention absorb materially 40 less moisture, are more resistant to corrosion, abrasion, and soil pressures, are of greater tensile and compressive strength than the saturated conduits heretofore known to me. Such conduits saturated with coal tar pitch are also more 45 resistant to attack by molds, fungi, and all cellulose-destroying organisms.

This application is a division of my co-pending application Serial No. 613,937 filed May 27, 1932.

It is to be understood that this invention is not 50 restricted to the present disclosure otherwise than defined by the appended claims.

I claim:

1. A batch process of impregnating fibrous conduits which comprises maintaining a body of saturant, drying a batch of said conduits, immersing the batch of dried conduits in the body of saturant, thereafter subjecting the conduits, while immersed in the saturant, to vacuum conditions, permitting the batch of conduits to soak in the 55 saturant while vacuum conditions are maintained on the saturant until the conduits are substantially completely saturated, interrupting the vacuum while maintaining the conduits immersed in the saturant to complete the saturation of the 60 conduits and removing the saturated conduits from the saturant.

2. A batch process of saturating fibrous conduits which comprises substantially continuously maintaining a body of saturant, successively immersing batches of dried conduits in said body of saturant, after each batch of dried conduits is 70 immersed in the saturant subjecting the body of saturant containing the immersed conduits to vacuum conditions and maintaining said vacuum 75

conditions until the conduits are substantially completely saturated, interrupting the vacuum while the conduits are immersed in the saturant, and increasing the pressure on the saturant to cause the entry of additional saturant into the conduit walls and complete the saturation of the conduits, and then removing the saturated conduits from the saturant.

3. A batch process of saturating fibrous conduits which comprises substantially continuously maintaining a body of bituminous saturant, successively immersing batches of dried conduits in said body of bituminous saturant, after each batch of dried conduits is immersed in the said saturant subjecting the body of said saturant containing the immersed conduits to vacuum conditions and maintaining said vacuum conditions until the conduits are substantially completely saturated, interrupting the vacuum while the conduits are immersed in the bituminous saturant, increasing the pressure on the said saturant to cause the entry of additional bituminous saturant into the conduit walls and complete the saturation of the conduits, and removing the saturated conduits from the said saturant.

4. A batch process of saturating fibrous conduits which comprises substantially continuously maintaining a body of coal tar pitch, successively immersing batches of dried conduits in said body of coal tar pitch, after each batch of dried conduits is immersed in the coal tar pitch subjecting the body of coal tar pitch containing the immersed conduits to vacuum conditions and maintaining said vacuum conditions until the conduits are substantially completely saturated, interrupting the vacuum while the conduits are immersed in the coal tar pitch, increasing the pressure on the said coal tar pitch to cause the entry of additional coal tar pitch into the conduit walls and complete the saturation of the conduits, and removing the saturated conduits from the coal tar pitch.

5. A batch process of saturating fibrous conduits which comprises immersing the conduits in a body of pitch saturant, while the conduits are immersed in the saturant subjecting them to vacuum conditions, soaking the conduits in the saturant while vacuum conditions are maintained thereon, interrupting the vacuum to cause the entry of additional saturant into the voids of the conduits to complete the saturation thereof,

and removing the saturated conduits from the saturant.

6. A batch process of saturating fibrous conduits which comprises immersing the conduits in a body of saturant from the group: coal tar pitch and water gas pitch, while the conduits are immersed in the saturant subjecting them to vacuum conditions, soaking the conduits in the saturant while vacuum conditions are maintained thereon, until substantially complete saturation of the conduits takes place, interrupting the vacuum to cause the entry of additional saturant into the voids of the conduits to complete the saturation thereof, and removing the saturated conduits from the saturant.

7. A batch process of saturating fibrous conduits initially containing air and moisture, comprising providing a hot body of heat liquefied bituminous saturant, immersing the conduits in the body of saturant and permitting them to soak under atmospheric pressure in the saturant until substantially dried, pulling a vacuum on the body of saturant containing the dried conduits and permitting the conduits to soak under vacuum conditions until substantially complete saturation of the conduits has occurred, interrupting the vacuum to complete the saturation of the conduits, and removing the saturated conduits from the body of saturant.

8. A process of waterproofing and strengthening absorbent conduits having relatively rigid walls of substantial thickness and density and constituted of organic fibrous material, the conduit walls initially containing air and moisture, comprising providing a hot bath of heat liquefied coal tar pitch saturant of the type produced by low-temperature distillation methods and having a relatively low free carbon content, drying the conduits to remove substantially all moisture, soaking the conduits in said hot bath of pitch while subjecting the bath to a vacuum, the conduits being immersed in the bath and the vacuum being initiated after the conduits have been wholly immersed, interrupting the vacuum after the conduits have become highly saturated, and continuing the soaking of the conduits, to substantially completely fill the voids in the walls of said conduits without producing substantial thermal decomposition of the fibrous material, and then removing the conduits from the bath.

GEORGE EMBERG.